

1

3,471,333

**METHOD OF UNPLUGGING FUEL-CELL OXYGEN INLETS AND THE LIKE**

Robert Lee Novack, Hanover, Mass., assignor to Prototech Company, division of Bolt Beranek and Newman Inc., Cambridge, Mass., a corporation of Massachusetts  
No Drawing. Filed Aug. 9, 1967, Ser. No. 659,295  
Int. Cl. H01m 27/00

U.S. CL. 136—86

4 Claims

**ABSTRACT OF THE DISCLOSURE**

A novel method is disclosed of unplugging oxide deposits in the region where electrochemical cell oxygen inlets contact the electrolytic medium involving the periodic introduction of a critical quantity of steam.

The present invention relates to methods of unplugging oxygen inlets in electrochemical cells and the like, being more particularly, though not exclusively, directed to methods of unplugging oxide deposits developed at the region where oxygen inlets to fuel cells and the like contact an elevated temperature substantially anhydrous electrolytic medium.

Particularly in anhydrous alkaline-hydroxide fuel cells and the like, wherein an oxidant such as oxygen or air (hereinafter generically referred to as oxygen) is introduced in the cathode region of the electrolytic medium, prolonged operation has been found to result in the lodging of oxide deposits apparently from the electrolytic medium or additives associated therewith at the region where the oxygen inlet contacts the electrolytic medium. While the cell may be shut down and the oxygen inlet unplugged, this is not a satisfactory solution for applications where continuous operation over long periods of time is required.

An object of the invention, accordingly, is to provide a new and improved method of unplugging such oxide deposits that is adapted to be used without substantially disrupting the continuous operation of the cell, without necessitating the shut down or disassembly of the cell, and without poisoning or otherwise destroying or modifying the efficacy of the electrolytic medium employed in the cell. In summary, this end is achieved through the periodic introduction of steam, preferably from a point external to the cell, of quantities sufficient to loosen the oxide deposits, but insufficient to change the water content or other properties of the electrolytic medium.

Other and further objects will be explained hereinafter and will be more particularly delineated in the appended claims.

Preferred cells subject to the above-described difficulties include 400°–600° C. substantially anhydrous molten alkaline-hydroxide electrolytic media provided with an anode, such as a palladium-containing hydrogen-permeable, but otherwise non-porous layer, and a preferably non-porous nickel cathode structure which may, indeed, comprise the cell housing, itself. Oxygen is fed into the medium in the cathode region to agitate the same and to insure the continual generation of peroxides and superoxides within the medium that serve as the cell oxidant, and with a barrier preferably interposed between the anode and cathode that is pervious to the ions of the electrolyte, but of sufficient dimensions and of sufficiently restricted porosity to prevent substantial agitation transfer from the oxygen-agitated cathode region to the anode region, as described, for example, in co-pending application of David Moulton, Robert Novack and Walter Juda, Ser. No. 539,768, filed Apr. 4, 1966,

2

for Fuel Cell Process and Apparatus. As described therein, cells of the above type are operated with the electrolytic medium in contact with an oxygen-containing atmosphere and at a temperature of at least substantially 300 degrees C. and sufficient to render the medium molten and substantially anhydrous, with the peroxide and superoxide functioning as substantially the sole fuel cell electrochemical oxidant to provide substantially the entire current output of the fuel cell.

In such cells, a convenient way of introducing the oxygen is by means of tubing, as, for example, of nickel, that bubbles oxygen into the region of the cathode structure. After several days of operation, however, it will customarily be noted that the inlet flow rate of the oxygen becomes decreased and, indeed, the power density of the cell drops off. This has been traced to oxide deposits that have been found to develop in such periods of time in the region of the inlet tube contacting the electrolytic medium, plugging the inlet. These deposits are extremely hard and difficult to remove, particularly during the continued high-temperature operation of the cell. Attempts, indeed, to snake a wire into the inlet tube to try to dislodge the plugging oxide deposits have proven ineffectual.

In accordance with the present invention, it has been found that these deposits may be rapidly loosened and bubbled away by the periodic introduction of steam at the plugged region. If, however, too much water vapor is introduced into the electrolytic medium, this will tend to destroy the substantially anhydrous state of the medium required for optimum peroxide and superoxide formation. It has been found that the introduction of steam must be controlled to provide a quantity only sufficient to loosen the oxide, but insufficient to cause the electrolyte medium at the inlet region to change its substantially anhydrous state.

As an example, in a cell operating with about 500 grams of 90 percent KOH and 10 percent NaOH as the electrolytic medium, maintained at a temperature of 475° C., and having hydrogen fuel applied through a platinum-containing anode layer and oxygen introduced in the form of air bubbled through a  $\frac{1}{8}$ -inch nickel tube at the cathode region at a rate of 500 ml./min., the air inlet flow rate and the power density will deteriorate as the result of such plugging within about four days of operation. If, in response to such degradation, at the end of each such period of time, one-to-two drops of water (about 0.05–0.1 ml.) are externally inserted into the oxygen inlet, it has been found that the water droplets become converted into steam in dropping through the inlet tube as the result of the elevated temperature of the cell, and fully loosen the oxide to unplug the inlet, but with insufficient residual water vapor resulting to alter the desired substantially anhydrous state of the electrolytic medium.

As another example, limited water vapor has been introduced into the air at the inlet, the steam being at a partial pressure of about 400 mm. of mercury (total pressure about 1 atmosphere), obtaining the satisfactory unplugging without substantially altering the anhydrous state of the electrolytic medium (about 500 grams) over about two minutes at an air-steam flow of 500 ml./minute.

Clearly, any well-known, water-mixing or droplet-introducing apparatus, such as mixers, syringes, or the like, may be employed and adapted either to operate periodically at fixed intervals of time or periodically in response to degradation of low rate or power density, by thoroughly well-known feed-back or sensing controls and techniques. Further, modifications will also occur to those skilled in this art.

What is claimed is:

1. A method of operating a fuel cell containing an alkali-metal hydroxide electrolyte medium with an oxygen inlet in contact therewith, that comprises maintaining the medium at a temperature in excess of about 300° C. and sufficient to render the medium molten and substantially anhydrous and in contact with an oxygen-containing atmosphere in an amount sufficient to provide in the medium at least one of alkali-metal peroxide and superoxide, said peroxide and superoxide functioning as substantially the sole fuel cell electrochemical oxidant, applying hydrogen-containing fuel to the fuel cell, drawing current from said fuel cell while holding the said medium at such temperature and while utilizing said oxidant electrochemically to provide substantially the entire current output of the fuel cell, whereby oxide deposits tend to plug said inlet region, and periodically introducing steam to the region of said oxygen inlet in contact with said medium in sufficient quantity to loosen the oxide at said inlet region but insufficient to cause the medium at said region to change its substantially anhydrous state.

2. A method as claimed in claim 1 and in which said steam is produced by water droplets introduced into the said inlet and vaporized in passing through the same into the elevated-temperature medium.

5. A method as claimed in claim 1 and in which said steam-introducing step is effected in response to degradation in at least one of inlet oxygen flow rate and power density.

10 6. A method as claimed in claim 1 and in which the elevated temperature is in excess of about 400° C.

#### References Cited

##### UNITED STATES PATENTS

|    |           |         |              |       |        |
|----|-----------|---------|--------------|-------|--------|
| 15 | 2,060,663 | 11/1936 | De Walt.     |       |        |
|    | 3,330,699 | 7/1967  | Tantram      | ----- | 136—86 |
|    | 3,350,226 | 10/1967 | Lieb et al.  | ----- | 136—86 |
|    | 3,403,056 | 9/1968  | Barde et al. | ----- | 136—86 |

20 WINSTON A. DOUGLAS, Primary Examiner

M. J. ANDREWS, Assistant Examiner